

## [54] SPECTRALLY SENSITIZED SILVER HALIDE PHOTOGRAPHIC EMULSIONS

[75] Inventors: **Yasuhiro Nakamura; Yoshiyuki Nakazawa; Tohru Sueyoshi; Akira Sato; Tadashi Ideda**, all of Kanagawa, Japan

[73] Assignee: **Fuji Photo Film Co., Ltd.**, Kanagawa, Japan

[22] Filed: **May 31, 1973**

[21] Appl. No.: **365,677**

## [30] Foreign Application Priority Data

May 31, 1972 Japan ..... 47-54497

[52] U.S. Cl. .... 96/120, 96/107

[51] Int. Cl. .... G03c 1/02

[58] Field of Search ..... 96/120, 107

## [56] References Cited

## UNITED STATES PATENTS

2,112,162 3/1938 Kendall ..... 96/120  
2,411,507 11/1946 Collins et al. .... 96/120

3,629,274 12/1971 Oliver ..... 96/120

Primary Examiner—J. Travis Brown

Attorney, Agent, or Firm—Sughrue, Rothwell, Mion, Zinn & Macpeak

## [57] ABSTRACT

A silver halide photographic emulsion containing at least one sensitizing dye represented by the general formula:



has high spectral sensitivity in the vicinity of 460 - 490 m $\mu$ . Moieties R<sub>1</sub> - R<sub>4</sub> are defined in the specification.

7 Claims, 1 Drawing Figure

PATENTED MAR 25 1975

3,873,323



# SPECTRALLY SENSITIZED SILVER HALIDE PHOTOGRAPHIC EMULSIONS

## BACKGROUND OF THE INVENTION

### 1. Field of the Invention

This invention relates to a silver halide photographic emulsion containing novel sensitizing dyes, and particularly to a silver halide photographic emulsion having a high spectral sensitivity in the vicinity of 460 - 490 m $\mu$ .

### 2. Description of the Prior Art

In the manufacturing of silver halide photographic emulsions it has been well known that when a sensitizing dye is added to the silver halide photographic emulsion the sensitive wave length region is expanded.

It has been well known that the spectrally sensitized wave length region and the spectral sensitivity of silver halide photographic emulsions containing sensitizing dyes are influenced by the chemical structure of the sensitizing dyes and, especially, by the kinds of hetero rings and the substituents on the sensitizing dyes.

Sensitizing dyes often display spectral sensitizations which are not expected at all due to a slight difference in chemical structure, and the sensitization due to the J-aggregate (J-band) of sensitizing dyes depends on the chemical structures of the sensitizing dyes.

The sensitization due to the J-aggregate of a sensitizing dye is effective for the spectral sensitization in the region of a specified wave length, and it is very important to develop sensitizing dyes which form the J-aggregate in order to highly sensitize a specified wave length region desired in the silver halide photographic sensitive material.

For example, the energy distribution of a light source used in the facsimile field has a peak in the vicinity of 480 m $\mu$ . Therefore, it is desirable that a photographic emulsion used in the facsimile art has a maximum sensitization in the vicinity of its peak, e.g., about 460 - 490 m $\mu$ .

However, there are little or no dyes which form the J-aggregate in the vicinity of 460 - 490 m $\mu$  and, if any do form the J-aggregate, the sensitivity thereof is too low.

## SUMMARY OF THE INVENTION

It has been found that new sensitizing dyes which are described in detail below are useful ones that form the J-aggregate and strongly spectrally sensitize the wave lengths region in the vicinity of 460 - 490 m $\mu$ .

The object of this invention is to provide a silver halide photographic emulsion having high spectral sensitivity in the vicinity of 460 - 490 m $\mu$ , and it has been accomplished by adding to a silver halide photographic emulsion novel sensitizing dyes of the following general formula (I):



wherein R<sub>1</sub> and R<sub>2</sub> each represents identical or different alkyl groups as are conventionally used in cyanine

dyes, i.e., both substituted and unsubstituted alkyl groups such as methyl, ethyl, n-propyl, n-butyl, carboxyalkyl (for example, carboxymethyl,  $\beta$ -carboxyethyl,  $\gamma$ -carboxypropyl,  $\delta$ -carboxybutyl, etc.), alkoxyalkyl groups (for example,  $\beta$ -methoxyethyl), hydroxyalkyl groups (for example,  $\beta$ -hydroxyethyl, etc.), acyloxyalkyl groups (for example,  $\gamma$ -acetoxypropyl), sulfoalkyl groups (for example,  $\beta$ -sulfoethyl,  $\gamma$ -sulfopropyl,  $\gamma$ -sulfovutyl,  $\delta$ -sulfovutyl, etc.), aralkyl groups (for example, benzyl, phenethyl, p-carboxyphenethyl), vinylmethyl; and R<sub>3</sub> and R<sub>4</sub> may be identical or different and each represents an acyl group, i.e., aromatic acyl group (e.g., benzoyl, etc.) or an aliphatic acyl group, preferably having up to 3 carbon atoms (e.g., acetyl, propionyl, etc.) or an alkoxy carbonyl group (for example, methoxycarbonyl, ethoxycarbonyl, etc.).

In the above formulae, most preferred are those wherein any alkyl moiety which is present contains up to 4 carbon atoms, except for the alkyl moiety of the alkoxy or alkoxy carbonyl group, which preferably contain up to 3 carbon atoms.

As defined in general formula (I), the features of sensitizing dyes used in this invention reside in the fact that they have a 5,6-dichlorobenzimidazole nucleus as a hetero ring and an acyl or alkoxy carbonyl group as the terminal group. Those dyes having such a chemical structure readily form the J-aggregate and are effective to increase the spectral sensitivity in the vicinity of 460 - 490 m $\mu$ .

## BRIEF EXPLANATION OF DRAWING

FIG. 1 shows spectral sensitivity curves, in which (a) shows the spectral sensitivity curve of a silver halide photographic emulsion containing sensitizing dye (I) used in this invention and (b) shows the spectral sensitivity curve of an otherwise identical emulsion where dye (I) is replaced with control sensitizing dye A.

## DETAILED DESCRIPTION OF THE INVENTION

Typical examples of the novel sensitizing dyes of general formula (I) which are used in this invention are shown below, with the proviso that the sensitizing dyes used in this invention are not restricted to these examples.

Dye 1



Dye 2





A typical synthesis example of a sensitizing dye used in this invention is as follows. Reference should also be made to the text "The Chemistry of Heterocyclic Compounds, The Cyanine Dyes and Related Compounds", Francis M. Hamer, Interscience Publisher.

Synthesis A of Ethyl-4-(5,6-dichloro-1,3-diethyl-2(1H)-benzimidazolylidene)-2-acetyl-2-butenoate (Dye 1)

5 g of 5,6-dichloro-1,3-diethyl-2-( $\beta$ -N-acetyl anilinovinylen) benzimidazolium iodide and 2.5 g (100 percent excess) of acetoacetic acid ethyl ester were dissolved in 6.0 ml of ethanol, 3 ml of triethylamine was added, the system heated for 1 hr. under reflux at atmospheric pressure, then cooled, and 300 ml of water added and the separated crystals subjected to suction. The residue was treated with active carbon and recrystallized two times from acetic acid ethyl ester to yield 3.0 g of dye crystals (mp: 192° – 194°C,  $\lambda_{max}^{MeOH}$  436 m $\mu$ ).

Other dyes can be synthesized readily by those skilled in the art with a synthetic method similar to the process as mentioned above merely by varying the starting materials.

The sensitizing dyes used in this invention can spectrally sensitize silver halide photographic emulsions and are especially effective to expand the sensitivity region of gelatino-silver halide photographic emulsions.

4

They can also sensitize silver halide photographic emulsions which contain gelatin derivatives such as acetylated gelatin, phthalated gelatin, etc., hydrophilic colloids other than gelatin derivatives such as cellulose ether, partially hydrolyzed cellulose, polyvinyl alcohol, polyvinyl pyrrolidone, copolymers of maleic anhydride and phthalic acid and other synthetic or natural hydrophilic high molecular substances. Generally speaking, any photographic binder can be used with success in the present invention.

As the silver halide photographic emulsion used in this invention, various kinds of silver salts such as silver bromide, silver iodobromide, silver chlorobromide, silver chloroidobromide, etc., can be used and especially silver bromide and silver iodobromide emulsions are used effectively. So long as the silver halide is photosensitive, it can be used with success in the present invention.

20 However, most preferred emulsions are those wherein the weight ratio of silver halide to binder is from about 4 : about 1 to about 1 : about 4.

The present invention is very effective when the silver halide used has particles which are normal or ultra fine grains (for example, those with an average particle diameter in number, measured by the projected area method, of less than about 0.1  $\mu$ ). The effect of this invention is more remarkable for the ultra fine grains.

25 For the preparation of sensitized silver halide photographic emulsions according to this invention, the sensitizing dye can be dissolved in a suitable solvent such as methanol, ethanol, methylcellosolve, etc., and added as solution to a silver halide photographic emulsion in the manner commonly used in this art. Suitable solvents are easily selected, the primary considerations entering into the selection of the solvent being that the solvent is easy to handle, inexpensive, does not harm photographic properties and is not injurious to the health. Organic solvents miscible with water are generally used.

30 The amount of sensitizing dye contained in a silver halide photographic emulsion can be varied within, for example, a range of about  $1 \times 10^{-3}$  to about  $1 \times 10^{-4}$  mol/mol of silver. Especially excellent results are obtained when the amount of sensitizing dye is about  $5.8 \times 10^{-4}$  mols/mol of silver.

35 Additionally, any known sensitizing dye may be added to the silver halide photographic emulsion according to this invention.

In the preparation of a silver halide photographic emulsion according to this invention, any commonly used chemical sensitizer, toner, film-hardener, anti-fogging agent, surface active agent, thickener, plasticizer, lubricant, development accelerator, color coupler, UV-absorbent, irradiation inhibitor, matting agent, etc., may be added at proportions as are common in this art using any general addition technique.

40 The silver halide photographic emulsion according to this invention may be coated by any technique commonly used in the art onto a suitable substrate such as, for example, glass, a film of cellulose derivatives (triethyl cellulose, etc.), a film of a synthetic resin (polyethylene terephthalate, etc.), baryta paper, a resin-coated paper, synthetic paper and the like. In short, any photographic substrate can be used with success in the present invention.

45 Several examples of preferred embodiments of the present invention are given below.

A given amount (8 ml per 100 g of emulsion) of a methanolic solution (1/1,000 mol of dye per liter of methanolic solution) of one of the above mentioned sensitizing dyes used in this invention was individually added to 100 g of a gelatino silver iodobromide emulsion (I: Br ratio 3.97 molar): ratio of silver halide: binder 1:2 (weight); silver halide particle size of 0.08  $\mu$ , which was prepared in a known method. 7 ml of the resulting silver halide photographic emulsion was coated on a glass plate of cabinet size and dried to prepare a sample.

The sample was exposed through a No. 2 filter (Fuji Photo Co., through which light of a wave length longer than 450  $\mu$  passes) with an optical wedge by means of a tungsten lamp having a color temperature of 2,666°K (2,000 lux, 20 seconds) and then developed at 20°C for 5 min with a liquid developer of the following formulation:

|                            |          |   |
|----------------------------|----------|---|
| Metol                      | 2.2      | g |
| Sodium sulfite             | 96       | g |
| Hydroquinone               | 8.8      | g |
| Anhydrous sodium carbonate | 56       | g |
| Potassium bromide          | 5        | g |
| Water to make              | 1 liter. |   |

In table 1, the spectral sensitivity, fog and maximum sensitization are shown for sensitizing dyes according to this invention as well as control sensitizing dyes. FIG. 1 shows the spectral sensitivity curve of dye (I) of this invention and of control dye A based upon the data derived in this example.

TABLE 1

| Ex. No. | Dye | Amount of Dye added (mol/mol-Ag) | Sensitization degree | Fog  | Maximum sensitization |
|---------|-----|----------------------------------|----------------------|------|-----------------------|
| 1       | 1   | $5.8 \times 10^{-4}$             | 800                  | 0.04 | 480 $\mu$             |
| 2       | 2   | do.                              | 400                  | 0.04 | 475-480 $\mu$         |
| 3       | 3   | do.                              | 750                  | 0.04 | 480 $\mu$             |
| 4       | 4   | do.                              | 350                  | 0.04 | 475 $\mu$             |
| 5       | 5   | do.                              | 600                  | 0.04 | 480 $\mu$             |
| 6       | 6   | do.                              | 650                  | 0.04 | 480 $\mu$             |
| Con-    | A   | do.                              | 100                  | 0.04 | 458 $\mu$             |
| Control | B   | do.                              | 120                  | 0.04 | 465-470 $\mu$         |
|         | C   | do.                              | 110                  | 0.04 | 465 $\mu$             |
|         | D   | do.                              | 120                  | 0.04 | 460 $\mu$             |

The spectral sensitivity is shown under the heading "Sensitization Degree" as a specific sensitivity where the sensitivity of sensitizing dye A used as a control is set as 100.

The chemical structures of the sensitizing dyes which were used as controls are as follows:



As is seen from the data in Table 1, the emulsions containing the sensitizing dyes according to this invention have a sensitization maximum within the range of 460 - 490  $\mu$  and show little fog and high sensitivity as compared with the controls.

FIG. 1 shows the spectral sensitivity curves of silver halide photographic emulsions which contain novel sensitizing dye (I) used in this invention and control sensitizing dye A, respectively.

As is seen from FIG. 1, sensitizing dye (I) used in this invention forms the J-aggregate and has a high spectral sensitivity at 460 - 490  $\mu$ .

While the invention has been described in detail and with reference to specific embodiments thereof, it will be apparent to one skilled in the art that various changes and modifications can be made therein without departing from the spirit and scope thereof.

What is claimed is:

1. A silver halide photographic emulsion characterized by containing at least one sensitizing dye represented by the following general formula:



wherein R<sub>1</sub> and R<sub>2</sub> each represents an alkyl or substituted alkyl radical selected from the group consisting of carboxyalkyl, alkoxyalkyl, hydroxyalkyl, acyloxyalkyl, sulfoalkyl and aralkyl, and R<sub>3</sub> and R<sub>4</sub> each represents an acyl or alkoxy carbonyl radical.

2. A silver halide photographic emulsion as claimed in claim 1 wherein R<sub>1</sub> and R<sub>2</sub> are unsubstituted alkyl.

3. A silver halide photographic emulsion as claimed in claim 1, wherein any alkyl moiety has up to 4 carbon atoms, with the exception of the alkyl moiety in the alkoxy group which has up to 3 carbon atoms.

4. A silver halide photographic emulsion as claimed in claim 3 wherein said acyl group is an aromatic acyl or aliphatic acyl group having up to 3 carbon atoms.

5. A silver halide photographic emulsion as claimed in claim 4 wherein said aromatic acyl group is benzoyl.

6. A silver halide photographic emulsion as claimed in claim 4 wherein said silver halide has an average particle diameter, in number, of less than about 0.1  $\mu$ .

7. A silver halide photographic emulsion as claimed in claim 1 wherein said sensitizing dye is present in an amount of from about  $1 \times 10^{-3}$  to about  $1 \times 10^{-4}$  mol-mol of silver.

\* \* \* \* \*